

Feb. 19, 1929.

1,702,600

W. F. GRUPE

# METHOD OF FORMING CORK DISKS AND GASKETS AND PRODUCT OF THE SAME

Filed Aug. 10, 1926

Fig. 1



Fig. 2.



Fig. 3. 25



INVENTOR,  
William F. Gryfe,  
BY  
Henry J. Lucke,  
ATTORNEY.

Patented Feb. 19, 1929.

1,702,600

# UNITED STATES PATENT OFFICE.

WILLIAM F. GRUPE, OF LYNDHURST, NEW JERSEY, ASSIGNOR TO BOUCHER CORK COMPANY, INC., OF NEW YORK, N. Y., A CORPORATION OF NEW YORK.

## METHOD OF FORMING CORK DISKS AND GASKETS AND PRODUCT OF THE SAME.

Application filed August 10, 1926. Serial No. 128,481.

This invention relates to a method of forming cork disks and gaskets and the product of the same.

It is well-known to those skilled in the art that such crown caps are substantially circular in form and are made of metal by punching operation. Within the seat of the crown cap, cushions of natural cork and of composition cork have heretofore been employed to serve as the sealing medium. However, in view of the continued high demands for natural cork for caps and other sealing purposes, and particularly in view of the restricted availability of less than twenty-five per cent imposed by nature of natural cork of the required quality capable in natural state of effecting perfect sealing, the attempt has been made to employ sealing disks of composition cork in substitution of natural cork. However, when composition cork (which is formed of cork granules bonded to one another by adhesives such as adhesives containing albumen, casein and the like) is brought in contact with the fluid contents of the bottle, the adhesive of the above nature is subject to decomposition and putrefaction, attended by discoloration of the cork due to the resulting chemical action, and consequent pollution of the contents of the bottle.

It has also been proposed to employ a collet of waxed paper or the like interposed between the disk of natural cork and the metal cap, but such procedure involves additional expense in material and in the assembly of the cap, and also gives rise to the penetration of the liquid through the pores and thence through the cork disk to the paraffin of the collet or to the paper itself where paraffin is not employed, and thus the flavor or odor of bottled contents is contaminated.

It has also been proposed to apply a sheet of lead or other metallic foil on the outer face of the cork disk, but this procedure enburdens the cost of additional material and the labor and machines for applying the metal foil to one face of each cork disk; furthermore, the metal foil reduces the sealing quality of the cork disk since the metal foil is interposed between the lip of the bottle and the cork disk.

The present invention is directed to the production of products of cork or like material, particularly from cork waste, whereby the product is substantially free from pores inherent in natural cork and possesses the

characteristics of sealing and like properties of natural cork, and bonded together autogenously and without the use of any adhesive or the character heretofore employed.

The present invention is particularly useful in the production of cushions of the disk and other forms for crown caps, also for gaskets for automotive engines and general sealing uses, and are also applicable for other uses in which natural cork is at present employed.

Pursuant to a preferred form of my invention for use as sealing cushions in crown seals for bottled beverages and for use as gaskets in the assembly of sealed motor parts, the aforesaid products are formed by charging into a mold of suitable contour particles of cork to the desired amount, subjecting the charge to the desired compression as by reducing the volume of the charge within the mold and then subjecting the compressed charge to an elevated temperature by applying the temperature solely on one side of the mold, that is to say, on one face of the charge, to thereby effect an increased baking effect on the cork particles at and closely adjacent such one face and securing a baking effect at and through the remainder of the charge sufficient to bind the cork particles to one another and close the pores of the cork particles and the interstices between the cork particles. The resulting product comprises a mass portion at one face of which the baking heat has been applied and constituted of cork substantially devoid of pores or other openings and devoid of clearances between the cork particles and which mass possesses a limited extent of resiliency or yieldability. The mass portion at the opposite face of the cork product is also devoid of pores or other openings and devoid also of any clearances between the cork particles and possesses a resiliency and yieldability of the character comparable to that of natural cork of the higher grades.

By the above procedure, the molded product may be in the form of a sheet, from which are punched in the usual manner circular disks or other forms of sealing media for crown caps and closures for bottles and other containers.

Gaskets of the desired configuration and provided with the usual openings for the reception of bolts and for affording communication for the requirements of a motor, as for gasket use between a carburetor and the en-

60

65

70

75

80

85

90

95

100

105

110

gine inlet manifold or between the parts of the water cooling system, or between the top or other plate and the body of the cylinders and all other gasket applications.

5 Further features and objects of the invention will be more fully understood from the following detail description and the accompanying drawing, in which

10 Fig. 1 is a central, vertical section of a diagrammatic form of mold, showing the stage of subjecting the compressed charge to a baking temperature pursuant to my invention;

15 Fig. 2 is a perspective view showing a portion of a mold sheet from which circular cushion disks are being punched; and

20 Fig. 3 is a detail sectional view on line 3—3 of Fig. 2.

25 Referring to Fig. 1, the mold 10 is of any desired shape and of any desired formation. The type of mold illustrated in Fig. 1 is of a simple form serving for the production of a sheet of the thickness comparable to that for forming circular disks for crown caps for sealing beverage bottles.

30 For simplicity of illustration, the mold shown in Fig. 1 may be provided with the upper or hopper portion 11 into which the cork particles are charged. The compression of the charge may be effected by means of the pressure plate 12, freely fitting within the four sides of the mold and subjected to a hydraulic or other pressure device. The quantity of the charge of cork particles is 35 determined by the extent of compression desired, which may range from a reduction in volume from two volumes to one volume and from six volumes to one volume.

40 A factor in determination of the extent of compression is the use to which the resulting product is to be applied. Generally speaking, the extent of compression determines the degree of "life" of the resulting product, particularly at the face of the product which is subjected to the lower temperature of baking, as will appear more fully hereinafter.

45 Upon compressing the charge 13 to the desired extent, the compression plate 12 is retained in position by any suitable means, as by one or more bars 14 passing through oppositely disposed openings 15, 16 in the sides 17, 18 of the mold hopper 11. Such procedure corresponds generally to steps of charging the mold and compressing the charge as is set forth in my copending application entitled Separators for storage batteries, Serial No. 749,396 and filed by me on the 19th day of November, 1924.

50 The nature of the charge may be any suitable form of cork. For commercial reasons, cork waste is desirable by reason of its low cost of production; and by reason of its ease of availability as a by-product attending the manufacture of the many commercial forms of cork at numerous locations other than the

countries of production of natural cork. Cork waste includes tapered cork waste resulting from the cutting of tapered cork stoppers, granulation of the left-over portions of sheets of natural cork from which sealing disks or gaskets or the like have been punched or cut. Cork waste also includes so-called cork wool and the unused portions of thin sheets of natural cork from which cigarette tips and the like have been sliced or cut. 75

75 The baking is carried out by means of any form of heating capable of attaining the desired temperature of baking. For the manufacture of sheets of a thickness suitable for forming sealing disks and motor gaskets, the 80 heating element is preferably of the electrically heating type as is indicated at 19, usually comprising a block of vitreous or artificial stone composition, in which is positioned or molded an electrical resistance wire 85 20, embedded in finely divided, insulating material 21, as will be understood by those skilled in the art.

85 Upon applying the heating face 22 of the heating block 19 to the under face 23 of the 90 mold 10, the baking heat is applied directly to the lower mass portion 24 of the charge 13. It should be observed that cork possesses a high coefficient of heat insulation and accordingly the rate of conduction of heat 95 energy through the cork charge is low, which property of cork and the absence of direct heating of the charge 13 other than on its lower face, effects a baking to a high degree of the lower mass portion 24 of the charge 13. 100 Such baking temperature, however, is insufficient to cause any substantial charring of the lower mass portion 24.

105 The range of baking temperature is dependent upon the period of baking and the period of baking is in turn dependent upon thickness of the charge within the mold. The usual range of baking temperature is from 150° C. to 275° C., within which range the distillation of the resins inherent in cork or 110 the added resins of similar nature takes place and effects the spaced localization by the resins on the surface of the cork particles.

115 The general effect of the baking pursuant to my invention is indicated in Fig. 3. The lower mass portion 24 assumes a decided darkened appearance as a result of the baking. The structure of the lower mass portion 24 is substantially that of the nature of 120 solidification upon cooling after attaining a slightly viscous or molten state. The mass portion 24 is substantially homogeneous and wholly free from pores and clearances between the original particles and the lines of demarkation of the original cork particles have been effaced. The texture and pliability and toughness of the back or lower mass portion 24 of my product is comparable to that of leather. 130

The constituency of the mass portion 25 at and adjacent the upper and less baked face of the molded product is that of a cork mass having the full "life" of natural cork of the 5 higher quality, namely, having the properties of resiliency and of permanence of formation and other characteristics of natural cork of the higher quality, affording repeated use as a sealing medium. The outer face of the 10 mass portion 25 is wholly devoid of pores and the clearances between the original particles are eliminated by the baking, which result is comparable to autogenous welding of metals. It will be appreciated that in the 15 simultaneous baking and compression of the cork charge, the resins inherent in natural cork are distilled at the successively increasing temperatures corresponding to their temperatures of volatilization, and that the relatively 20 tougher portions of natural cork such as the walls of the original cells are gradually broken down as the temperature increases. The distribution of the distilled resins through the mass effectually closes the pores 25 of the cork particles and this action takes place within the intermediate portion 26 and the uppermost portion 25 of my product where the temperature is not sufficient to 30 produce the nature of solidification of the lowermost portion 24. It will be observed that such resins are wholly inert and wholly immune toward water, beverages and including any alcoholic content, and for the purpose of the present invention are highly advantageous in that no odor or flavor of whatsoever character is imparted to the contents of the bottle.

If desired, rosin or other resin of the nature of resins natural in corkwood may 40 be added to the charge.

As is indicated in Fig. 2, the resulting sheet 30 is punched to form circular or other shapes of disks 31 of the proper diameter to serve as sealing disks in crown caps or the like. 45 The punching openings are indicated at 32, 33. In a similar manner, gaskets for automobile parts and for general gasket use may be punched from such sheets 30.

In the use of disks or other forms of my 50 product for bottle sealing cushions the disks may be steamed or boiled to remove any loose or charred portions, and also to wholly eliminate all tendency to leave any dark "soot" on the fingers of the operator when handling the 55 disks or on other materials with which they are brought into contact.

By selecting the depth or other corresponding dimension of the mold to conform to the 60 dimension of the resulting baked product, the opposite faces of the product are therefore molded, that is to say, the material at each molded face possesses a continuous surface of cork and bonded continuously and substantially uniformly by the resin inherent 65 in cork when such resin is used alone as the

binder, or by such cork resin together with any additional resin added to the charge of the mold. The material at such molded surfaces has a texture comparable to that of leather, that is to say, resists mechanical 70 abrasion and has an increased resistance against permeation by liquids, moisture, lubricating oils in liquid or vapor form and the like as compared with a surface formed by severing the molded product. 75

Whereas, I have described my invention by reference to specific forms thereof, it will be understood that many changes and modifications may be made without departing from the spirit of the invention. 80

I claim:

1. The method of forming baked, compressed cushions, gaskets and like products of cork, which comprises compressing cork particles in a mold to a desired shape, baking 85 the compressed cork particles by applying a higher temperature to one side of the mold than on another side of the mold, said higher temperature being capable of effecting the vaporization of the resin inherent in the cork 90 particles, and forming the product from the resulting baked product.

2. The method of forming baked, compressed cushions, gaskets and like products of cork, which comprises compressing cork 95 particles in a mold to a desired shape, baking the compressed cork particles by applying a higher temperature to one side of the mold than on another side of the mold, said higher temperature being capable of effecting the vaporization of the resin inherent in the cork particles, and forming the product from the resulting baked product by punching operations. 100

3. The method of forming baked, compressed cushions, gaskets and like products of cork, which comprises compressing cork particles in a mold to a desired shape and of a thickness substantially that of the desired product, baking the compressed cork particles 105 by applying a higher temperature to one side of the mold than on another side of the mold, said higher temperature being capable of effecting the vaporization of the resin inherent in the cork particles, and forming the product 110 from the resulting baked product.

4. The method of forming baked, compressed cushions, gaskets and like products of cork, which comprises compressing cork particles in a mold to a desired shape and of a thickness substantially that of the desired product, baking the compressed cork particles by applying a higher temperature to one side of the mold than on another side of the mold, said higher temperature being capable 125 of effecting the vaporization of the resin inherent in the cork particles, and forming the product from the resulting baked product by punching operations.

5. A cushion, gasket or like product formed 130

of compressed cork baked at one side to a greater maturity than on the opposite side, the material at said opposite side being of greater resiliency than the material at said one side.

6. A cushion, gasket or like product formed of compressed cork baked at one side to a greater maturity than on the opposite side, the material at said opposite side being of greater resiliency than the material at said one side, the opposite faces of said product being molded.

7. A cushion, gasket or like substantially

flat product formed of baked, compressed cork particles, the resiliency at one flat face 15 being greater than the resiliency at the opposite flat face.

8. A cushion, gasket or like substantially flat product formed of baked, compressed cork particles, the resiliency at one flat face 20 being greater than the resiliency at the opposite flat face, said flat faces being of molded formation.

In testimony whereof I have signed this specification this 9th day of August, 1926.

WILLIAM F. GRUPE.